# EUROPEAN PATENT APPLICATION

(11) **EP 4 767 839 A1**
(43) Date of publication of application: **01.07.2026**
(21) Application number: 24887280.6
(22) Date of filing: 01.04.2024
(51) Int. Cl.: A24B 15/167

(54) **AEROSOL-GENERATING SUBSTRATE AND PREPARATION METHOD THEREFOR**

(30) Priority: 06.11.2023 CN 202311466006
(71) Applicant: Humble Grace Limited, Kowloon, Hong Kong (HK)
(72) Inventor: HAI, Tao, Kowloon (HK); WU, Ping, Kowloon (HK); YANG, Zhiquan, Kowloon (HK)
(74) Representative: Manitz Finsterwald Patent- und Rechtsanwaltspartnerschaft mbB
(86) International application number: PCT/CN2024/085368
(87) International publication number: WO 2025/097656

(57) **Abstract**

A method for preparing an aerosol generation substrate includes: preparing a substrate precursor: taking pretreated tobacco and/or an aromatic plant, an inorganic porous material, a polyol aerosol-forming agent, a flavor additive, and a binder, adding water and/or ethanol, and performing slurry preparation, granulation, and preliminary drying to form a basic particle; performing pressing and forming: to form an aerosol generation substrate with an air channel hole; and performing drying and puffing treatment: performing secondary drying and puffing treatment, where a wall material of the aerosol generation substrate is of a porous skeleton structure including continuous micropores. The preparation method does not require a plurality of times of high-temperature treatment, preventing destruction of flavor by high temperatures. The wall material forms the porous skeleton structure including the continuous micropores. This ensures structural strength and increases a contact area between external air and aerosol, so that the aerosol is more evenly mixed and the aerosol is abundant during inhalation. Additionally, an aerosol generation substrate prepared by using this method is provided.

## Description

This application claims priority to Chinese Application No. 202311466006.3, filed on November 6, 2023, and entitled "AEROSOL GENERATION SUBSTRATE AND PREPARATION METHOD THEREFOR", which is incorporated herein by reference.

### TECHNICAL FIELD

This application relates to the field of heat-not-burn atomization technologies, and in particular, to an aerosol generation substrate and a preparation method therefor.

### BACKGROUND

A heat-not-burn cigarette generates aerosol by heating an aerosol-generating section (an aerosol generation substrate) of the cigarette. The aerosol generated by the cigarette has a relatively good taste acceptance. However, a currently commercialized heat-not-burn cigarette often suffers from an insufficient aerosol volume. This is mainly because a tobacco sheet or another aromatic plant sheet used as the aerosol generation substrate undergoes a plurality of times of high-temperature treatment during a production procedure. Consequently, a flavor substance, a flavor additive, an aerosol-forming agent, and the like in tobacco or another aromatic plant are destroyed by high temperatures, affecting the taste.

### SUMMARY

A technical problem to be resolved in this application is to provide an improved aerosol generation substrate and a preparation method therefor.

A technical solution used in this application to resolve a technical problem thereof is to provide a method for preparing an aerosol generation substrate, including the following steps:
preparing a substrate precursor:
taking aroma-producing pretreated tobacco and/or an aromatic plant, an inorganic porous material, a polyol aerosol-forming agent, a flavor additive, and a binder, adding a pretreated thermally conductive material or electromagnetic induction material, adding a solvent, where the solvent is water and/or ethanol, and performing slurry preparation, granulation, and preliminary drying to form a basic particle, thereby obtaining the substrate precursor;
performing pressing and forming: adding the substrate precursor to a mold, and performing pressing and demolding, to form a substrate intermediate with at least one air channel hole; and
performing drying and puffing treatment: performing secondary drying and puffing treatment on the substrate intermediate formed in the step of performing pressing and forming to form an aerosol generation substrate, where a wall material of the aerosol generation substrate is of a porous skeleton structure including continuous micropores.

In some embodiments, in the step of preparing a substrate precursor, aromatic plants include at least one of plants of the following families: Liliaceae, Cupressaceae, Valerianaceae, Primulaceae, Fabaceae, Ericaceae, Annonaceae, Burseraceae, Mimosaceae, Iridaceae, Scrophulariaceae, Gentianaceae, Verbenaceae, Aristolochiaceae, Magnoliaceae, Oleaceae, Rosaceae, Solanaceae, Rubiaceae, Lauraceae, Rutaceae, Asteraceae, Orchidaceae, Poaceae, Piperaceae, Juglandaceae, Caprifoliaceae, Zingiberaceae, Apiaceae, Moraceae, Amaryllidaceae, Pinaceae, Usneaceae, Myrtaceae, Hamamelidaceae, and Malvaceae.

In some embodiments, in the step of preparing a substrate precursor, a viscosity of the formed basic particle is 500 Pa·s-1500 Pa·s, and a mass percentage content of a liquid phase component in the substrate precursor is 10%-50%.

In some embodiments, in the step of preparing a substrate precursor, pretreatment of the tobacco and/or the aromatic plant includes taking the tobacco and/or the aromatic plant for impact crushing treatment; and then placing the foregoing materials in a vacuum-sealed environment, adding an acidic treatment solution, and performing heating treatment at a heating temperature of 60°C-120°C, so that a volume of the tobacco and/or the aromatic plant expands by 1.1-1.5 times, and an amount of released free nicotine increases by at least 50%.

In some embodiments, in the step of preparing a substrate precursor, the inorganic porous material includes at least one of zeolite, molecular sieve, diatomaceous earth, montmorillonite, alumina, silica gel, activated carbon, calcium silicate, a chitosan porous material, a cellulose fiber, a lignin particle, clay, sepiolite, or palygorskite; and/or, the polyol aerosol-forming agent includes at least one of glycerol, propylene glycol, butylene glycol, and butanetriol; and/or, the flavor additive is an extract of tobacco and/or an extract of an aromatic plant; and/or, the binder includes one or a combination of a plurality of pullulan, tamarind polysaccharide, and hydroxypropyl methylcellulose.

In some embodiments, in the step of preparing a substrate precursor, the preparation of the substrate precursor includes the following raw materials in parts by mass: 30-80 parts of the tobacco and/or the aromatic plant, 10-30 parts of the polyol aerosol-forming agent, 0-5 parts of the binder, 5-20 parts of the inorganic porous material, and 5-10 parts of the flavor additive.

In some embodiments, in the step of preparing a substrate precursor, 0-8 parts by mass of an electromagnetic induction material are further added, where the electromagnetic induction material is at least one of iron, nickel, copper, germanium, carbon, chromium, tin, manganese, and aluminum.

In some embodiments, in the step of preparing a substrate precursor, 0-8 parts by mass of a resistance heating material are further added, where the resistance heating material includes at least one of zirconia, a carbon nanotube, nickel, chromium, and iron.

In some embodiments, in the step of preparing a substrate precursor, 0-5 parts by mass of a thermally conductive material subjected to high-temperature purification treatment are added, where the thermally conductive material is at least one of iron powder, copper powder, graphite powder, graphene, boron nitride, alumina, and carbon powder.

In some embodiments, in the step of performing drying and puffing treatment, low-temperature vacuum drying and puffing is adopted, and the solvent in a system overflows in an order of boiling points under low-temperature vacuum to form pores, so that the wall material of the aerosol generation substrate forms the porous skeleton structure including the continuous micropores.

In some embodiments, process parameters of low-temperature vacuum drying and puffing are: a temperature of 30°C-80°C, and a pressure of 15 kPa-85 kPa.

In some embodiments, in the step of performing drying and puffing treatment, hot-air drying and puffing is adopted, and the solvent in a system overflows in an order of boiling points under a hot-air drying condition to form pores, so that the wall material of the aerosol generation substrate forms the porous skeleton structure including the continuous micropores.

In some embodiments, when the solvent added in the step of preparing a substrate precursor is water, in the step of performing drying and puffing treatment, a freeze-drying process is adopted, and an aqueous ice crystal is transformed into a free water molecule through sublimation drying to overflow to form pores, so that the wall material of the aerosol generation substrate forms the porous skeleton structure including the continuous micropores.

In some embodiments, in the step of performing pressing and forming, by feeding the substrate precursor into the mold, under an action of a pressure, a compression polymer volume ratio is 6:1-10:3, an integrally formed substrate intermediate is demolded, there is at least one vertical rod in lower punch space of the mold, and an axial air channel hole adapted to a shape of the rod is pressed out after pressing of the upper punch.

In some embodiments, in the step of performing drying and puffing treatment, the formed micropore of the aerosol generation substrate is of 10 nm-20 µm, and a porosity is 20%-80%.

This application further provides an aerosol generation substrate, the aerosol generation substrate has at least one axial air channel hole, a wall material of the aerosol generation substrate is of a porous skeleton structure including continuous micropores, an aperture of the micropore is 50 nm-20 µm, and a porosity is 20%-80%.

In some embodiments, the aerosol generation substrate includes the following raw materials in parts by mass: 30-80 parts of tobacco and/or an aromatic plant, 10-30 parts of a polyol aerosol-forming agent, 0-5 parts of a binder, 5-20 parts of an inorganic porous material, and 5-10 parts of a flavor additive.

The implementation of this application has the following beneficial effects: For the aerosol generation substrate in this application, a pore-forming agent such as water and/or ethanol is added to the substrate precursor, pressing and forming is performed after preliminary drying, and then secondary drying and puffing treatment is performed, so that the water and/or ethanol in the wall material overflows, and in this case, continuous tiny pores are formed at an original location of the water and/or ethanol. The micropores are randomly arranged and interconnected, so that the wall material forms the porous skeleton structure including the continuous micropores. This ensures that the wall material has structural strength and increases a contact area between external air and aerosol, thereby implementing more even mixing. In addition, the preparation method in this application does not require a plurality of high-temperature treatment processes, and a reaction condition is relatively mild and easy to control. This prevents high temperatures from destroying a flavor substance, a flavor additive, an aerosol-forming agent, and the like in tobacco or another aromatic plant, and taste is mellower, thereby improving taste experience of the user.

### BRIEF DESCRIPTION OF DRAWINGS

The above and other purposes, features, and advantages of this application will become clearer by describing in more detail the example implementations of this application in conjunction with the accompanying drawings.
FIG. 1 is a schematic flowchart of a method for preparing an aerosol generation substrate according to an embodiment of this application; and
FIG. 2 is a scanning electron microscope image of an aerosol generation substrate according to Embodiment 1 of this application.

### DESCRIPTION OF EMBODIMENTS

Implementations of this application are described below with more details with reference to the accompanying drawings. Although embodiments of this application are shown in the accompanying drawings, it should be understood that this application may be implemented in various forms and should not be limited by the implementations described herein. On the contrary, these implementations are provided to make this application more thorough and complete, and to fully convey the scope of this application to a person skilled in the art.

A method for preparing an aerosol generation substrate in some embodiments of this application is shown in FIG. 1 and includes the following steps:
S1. Prepare a substrate precursor: taking pretreated tobacco and/or an aromatic plant, an inorganic porous material, a polyol aerosol-forming agent, a flavor additive, and a binder, adding a solvent, and performing slurry preparation, granulation, and preliminary drying to form a basic particle.

The solvent is water and/or ethanol. A viscosity of the basic particle is 500 Pa·s-1500 Pa·s, and a mass percentage content of a liquid phase component in the substrate precursor is 10%-50%, thereby obtaining the substrate precursor. The "mass percentage content of a liquid phase component" herein refers to a mass percentage content of a liquid phase in a solid substrate precursor.

For example, the viscosity of the basic particle is controlled at 500 Pa·s, 600 Pa·s, 700 Pa·s, 800 Pa·s, 900 Pa·s, 1000 Pa·s, 1100 Pa·s, 1200 Pa·s, 1300 Pa·s, 1400 Pa·s, 1500Pa·s, or the like. This is not specifically limited, for subsequent processing. A mass percentage of a liquid phase component in a dried substrate precursor is controlled at 10%, 12%, 14%, 15%, 16%, 17%, 18%, 20%, 25%, 30%, 35%, 40%, 45%, 50%, or the like. This is not specifically limited, for subsequent molding processing.

In an embodiment, the tobacco and/or the aromatic plant are aerosol-generating materials. For example, the tobacco and/or the aromatic plant are powder materials, to be mixed and filled with other components. The aromatic plant is a plant having a specific aroma, a specific medicinal value, or a specific physiological satisfaction effect. Aromatic plants include, but are not limited to, at least one of plants of the following families: Liliaceae (for example, Aloe vera, Allium sativum, Convallaria majalis, Hyacinthus orientalis, Allium cepa, and Smilax china), Cupressaceae (for example, Platycladus orientalis, Juniperus chinensis, Juniperus rigida, and Juniperus communis), Valerianaceae (for example, Nardostachys jatamansi, Valeriana officinalis, and Valeriana jatamansi), Primulaceae (for example, Lysimachia foenum-graecum and Lysimachia sikokiana), Fabaceae (for example, Amorpha fruticosa, Sindora glabra, Acacia farnesiana, Trifolium, Trigonella foenum-graecum, Glycyrrhiza uralensis, Acacia dealbata, Arachis hypogaea, Cassia angustifolia, Tamarindus indica, Dipteryx odorata, and Melilotus officinalis), Ericaceae (for example, Rhododendron capitatum, Rhododendron dauricum, Ilex, and Gaultheria leucocarpa), Annonaceae (for example, Cananga odorata, Artabotrys hexapetalus, and Cananga odorata var. fruticosa), Burseraceae (for example, Canarium album, Commiphora myrrha, and Boswellia), Mimosaceae (for example, Acacia catechu), Iridaceae (for example, Iris pallida, Crocus sativus, and Iris tectorum), Scrophulariaceae (for example, Verbascum thapsus, and Limnophila rugosa), Gentianaceae (for example, Swertia chirata, Gentiana scabra, and Menyanthes trifoliata), Verbenaceae (for example, Caryopteris incana, Vitex negundo, Vitex trifolia, Caryopteris mongholica, Caryopteris trichosphaera, Verbena officinalis, and Lippia citriodora), Aristolochiaceae (for example, Asarum heterotropoides, Asarum sieboldii, Aristolochia serpentaria, and Aristolochia delavayi), Magnoliaceae (for example, Illicium verum, Michelia alba, Michelia champaca, Magnolia liliiflora, and Illicium simonsii), Oleaceae (for example, Syringa, Jasminum officinale, Jasminum sambac, Osmanthus fragrans, Syringa reticulata, and Jasminum grandiflorum), Rosaceae (for example, Rosa rugosa, Armeniaca vulgaris, Malus pumila, Cerasus pseudocerasus, Rosa chinensis Crimson Glory, Crataegus pinnatifida, Prunus domestica, Rubus idaeus, Fragaria × ananassa, and Rosa banksiae), Solanaceae (for example, Capsicum annuum, Nicotiana tabacum, and Cestrum nocturnum), Rubiaceae (for example, Coffea arabica and Gardenia jasminoides), Lauraceae (for example, Cinnamomum glanduliferum, Cinnamomum porrectum, Laurus nobilis, Lindera glauca, Lindera aggregata, Litsea cubeba, Citrus aurantium, Litsea populifolia, Cinnamomum zeylanicum, Cinnamomum bodinieri, Cinnamomum wilsonii, Neocinnamomum delavayi, Cinnamomum septentrionale, Cinnamomum petrophilum, Sassafras tzumu, Cinnamomum burmannii, Cinnamomum tamala, and Cinnamomum subavenium), Rutaceae (for example, Citrus limon, Citrus sinensis, Citrus trifoliata, Adenosma indianum, Cinnamomum cassia, Citrus bergamia, Dictamnus dasycarpus, Citrus paradisi, Citrus medica var. sarcodactylis, Citrus reticulata, Murraya exotica, Ruta graveolens, Zanthoxylum bungeanum, Citrus junos, Citrus aurantifolia, Citrus aurantium, Citrus wilsonii, Citrus medica, Fortunella margarita, Citrus limonia, and Zanthoxylum armatum), Asteraceae (for example, Artemisia annua, Artemisia capillaris, Artemisia mongolica, Artemisia argyi, Atractylodes lancea, Cichorium intybus, Chrysanthemum morifolium, Aucklandia lappa, Taraxacum mongolicum, Inula helenium, Erigeron canadensis, Helichrysum arenarium, Calendula officinalis, Tagetes erecta, Tagetes patula, Tanacetum vulgare, Achillea millefolium, Blumea balsamifera, and Chromolaena odorata), Orchidaceae (for example, Cymbidium sinense and Vanilla planifolia), Poaceae (for example, Hierochloe odorata, Vetiveria zizanioides, Cymbopogon citratus, Cymbopogon goeringii, Cymbopogon tortilis, Cymbopogon distans, Cymbopogon nardus, Zea mays, Cymbopogon winterianus, Hordeum vulgare, and Saccharum officinarum), Piperaceae (for example, Piper kadsura, Piper nigrum, Piper arboricola, and Piper betle), Juglandaceae (for example, Carya cathayensis and Juglans regia), Caprifoliaceae (for example, Sambucus williamsii and Lonicera japonica), Betulaceae (for example, Betula lenta and Betula platyphylla), Zingiberaceae (for example, Amomum villosum, Kaempferia galanga, Elettaria cardamomum, Alpinia officinarum, Zingiber officinale, Alpinia galanga, Curcuma longa, Curcuma phaeocaulis, Amomum tsaoko, and Kaempferia galanga), Apiaceae (for example, Foeniculum vulgare, Anethum graveolens, Coriandrum sativum, Ligusticum jeholense, Daucus carota, Sium suave, Angelica sinensis, Pimpinella anisum, Sanicula chinensis, Torilis japonica, Bupleurum scorzonerifolium, Bupleurum chinense, Apium graveolens, and Anethum sowa), Moraceae (for example, Ficus carica, and Humulus lupulus), Amaryllidaceae (for example, Narcissus tazetta and Polianthes tuberosa), Pinaceae (for example, Pinus koraiensis, Pinus massoniana, Tsuga, Abies nephrolepis, and Pinus roxburghii), Usneaceae (for example, Usnea and Evernia prunastri), Myrtaceae (for example, Santalum album, Pterocarpus santalinus), Hamamelidaceae (for example, Eucalyptus citriodora, Syzygium aromaticum, Eucalyptus globulus, Eucalyptus robusta, Psidium guajava, Myrtus communis, Pimenta dioica, Chloranthus spicatus, Chloranthus fortunei, Chloranthus elatior, Liquidambar formosana, and Liquidambar orientalis), and Malvaceae (for example, Althaea officinalis, Abelmoschus moschatus, and Hibiscus sabdariffa). This is not specifically limited herein. Flowers, fruits, roots, stems, leaves, bark, seeds, and other parts of other naturally scented plants may also be used as the aromatic plants.

In step S1, the tobacco and/or the aromatic plant are subjected to aroma-producing treatment. The aroma-producing treatment includes the following steps: taking the tobacco and/or the aromatic plant and performing impact crushing treatment. The crushing treatment enables the material to become a particle in a shape of a spindle and/or a polyhedron. An aspect ratio of the spindle or the polyhedron is (3-5):1. For example, the aspect ratio is 3:1, 4:1, or 5:1. This is not specifically limited. Crushing is performed to obtain a particle in such a structure and with such an aspect ratio. When being in a shape of a spindle or a polyhedron, the tobacco, the aromatic plant, or a mixture of the two is more conveniently filled in the aerosol generation substrate. Another component may be filled in a gap in the tobacco, the aromatic plant, or the mixture of the two, thereby improving utilization of space in the substrate precursor. Because the substrate precursor is relatively compact, and all components are tightly filled in the substrate precursor in a manufacturing process, all the components are fixed in the substrate precursor without displacement. This is conducive to maintaining structural stability of the substrate precursor. This facilitates a subsequent preparation of the aerosol generation substrate, and implements a more robust overall structure and an improved aerosol formation effect.

The crushed tobacco and/or the aromatic plant are placed in a vacuum-sealed environment, treated with an acidic treatment solution, and then subjected to heating and aroma-producing treatment at a heating temperature of 60°C-120°C to obtain an aroma-containing material. When an acidic treatment solution is added, it is ensured that the acidic treatment solution fully wets the tobacco and/or the aromatic plant. A purpose of this wetting is to enable an acid solution to combine with nicotine inside cells and another alkaline flavor substance. After heating, a bound state is transformed into a free state, thereby adhering to surfaces of tobacco shreds and rapidly releasing during heating and inhalation. Therefore, final pH of a treatment system is 6.5-7.8. For example, pH is 6.5, 6.6, 6.7, 6.8, 6.9, 7.0, 7.1, 7.2, 7.3, 7.4, 7.5, 7.6, 7.7, or 7.8. This is not specifically limited. An amount of released free nicotine (monomeric nicotine) increases by at least 50%. Nicotine is converted from a bound state to a free state through heating. For example, most nicotine in tobacco is in a form of nicotine citrate, and can be decomposed into free nicotine and citric acid through heating, thereby reducing irritation and improving taste experience. The acidic treatment solution includes at least one of citric acid, benzoic acid, lactic acid, levulinic acid, salicylic acid, and tartaric acid. The foregoing acidic treatment solution is added to make reaction with the free nicotine gentler, so that another component in the tobacco, the aromatic plant, or the mixture of the two is not destroyed. For example, the heating temperature is controlled to be 60°C, 70°C, 75°C, 80°C, 90°C, 95°C, 100°C, 105°C, 110°C, 115°C, and 120°C. This is not specifically limited. The heating temperature is relatively mild, which prevents the flavor substance from being evaporated due to an excessively high temperature and avoids damage to the flavor substance by a high temperature. Through a combination of the crushing treatment and mild vacuum heating, cells in the tobacco and/or the aromatic plant are cavitated, thereby disrupting cell walls and transferring flavor substances inside the cells to surfaces. In this way, during heat-not-burn, aroma is more easily released, and flavor is richer and mellower, thereby improving taste experience of a user. For example, an added aroma-producing material is tobacco. An aroma test is conducted on tobacco before and after aroma-producing treatment. Contents of furfural and furfuryl alcohol in reacted tobacco are detected. Component contents of these two kinds of aroma in untreated tobacco are separately zero. After the aroma-producing treatment is performed, the contents of furfural and furfuryl alcohol respectively reach at least 0.15% and 0.25%. In other words, the aroma-producing treatment is performed on the tobacco and/or the aromatic plant, so that aroma can be more easily released, and flavor is richer and mellower, thereby improving taste experience of the user.

The inorganic porous material includes at least one of zeolite, alumina, silica gel, activated carbon, calcium silicate, a chitosan porous material, a cellulose fiber, a lignin particle, clay, sepiolite, and molecular sieve. The foregoing material is used as a porous aroma-carrying material. Based on a porous property of the porous aroma-carrying material, This is conducive to releasing aerosol. The inorganic porous material can absorb a large amount of flavor substances by using a pore structure of the inorganic porous material. In addition, adsorption performance and release performance of the porous material are affected by a temperature. When the temperature is relatively low, the release performance of the porous material is low. Therefore, in a processing or transportation stage after aroma enhancement, a flavor substance with a low boiling point can be better stored in the porous material, thereby preserving the aroma and prolonging a shelf life of a product. As a temperature increases in a heating and inhalation procedure, a flavor substance in the porous structure is slowly released, thereby achieving a sustained-release and aroma-enhancing effect, to ensure that an aerosol amount and aroma quality are consistent in an initial stage of inhalation and a final stage of inhalation.

The polyol aerosol-forming agent includes at least one of glycerol, propylene glycol, butylene glycol, and butanetriol. The flavor additive is an extract of tobacco and/or an extract of an aromatic plant, or another essence, fragrance, or the like. The flavor additive is added so that flavor of aerosol can be enriched, thereby improving experience of the user. The binder includes one or a combination of a plurality of pullulan, tamarind polysaccharide, and hydroxypropyl methylcellulose. The binder is added so that viscosity of substances in the system can be improved, and This is conducive to subsequent tableting. The presence of the binder and the inorganic porous material can effectively ensure an addition amount of tobacco and/or an aromatic plant, so that an aerosol amount of the aerosol generation substrate is sufficient. In addition, under an aqueous condition, the polyol aerosol-forming agent combines with exposed hydroxyl groups in the binder through hydroxyl groups, and water molecules in a dispersion system are accordingly transformed into a bound state. An overall state of a mixture changes from a liquid state to a solid state. The solid mixture is then mixed with another powder material to form a slurry. This facilitates granulation, pressing and forming, and subsequent formation of the porous skeleton structure by the wall material.

In a specific embodiment, in step S1, 0-5 parts by mass of a thermally conductive material subjected to high-temperature purification treatment are further added. For example, the parts by mass of the thermally conductive material are controlled to be 0 parts, 0.1 parts, 0.5 parts, 1 part, 2 parts, 3 parts, 4 parts, and 5 parts. This is not specifically limited. The thermally conductive material is added so that heating uniformity and thermal conductivity efficiency are improved, thereby improving heating uniformity and aerosol-generating utilization of the tobacco, the aromatic plant, or the mixture of the two. The thermally conductive material includes at least one of graphite powder, graphene, boron nitride, alumina, or carbon powder. A thermal conductivity coefficient of the thermally conductive material is 1 W/(m·k)-500 W/(m·k). For example, the thermal conductivity coefficient of the thermally conductive material is controlled to be 1 W/(m·k), 50 W/(m·k), 100 W/(m·k), 150 W/(m·k), 180 W/(m·k), 200 W/(m·k), 250 W/(m·k), 280 W/(m·k), 300 W/(m·k), 400 W/(m·k), or 500 W/(m·k). The above thermally conductive materials have high thermal conductivity performance, which enables rapid heating during inhalation of the user, so that heat is rapidly conducted to the tobacco, the aromatic plant, or the mixture of the two, and the tobacco, the aromatic plant, or the mixture of the two is enabled to produce aerosol, thereby generating aerosol. In an embodiment of this application, a particle size of a selected thermally conductive material is 20 nm-2 µm. For example, the particle size of the selected thermally conductive material is 20 nm, 30 nm, 50 nm, 80 nm, 90 nm, 100 nm, 200 nm, 300 nm, 400 nm, 500 nm, 600 nm, 700 nm, 900 nm, 1 µm, 1.5 µm, or 2 µm. This is not specifically limited. The particle size of the thermally conductive material is controlled to be within the foregoing disclosed range, thereby being conducive to uniform thermal conduction of the thermally conductive material.

A porosity of the thermally conductive material is >65%. Under a condition of a high porosity, pores of the thermally conductive material can adsorb more polyol aerosol-forming agents and tobacco/aromatic plant products to improve heat conversion, thereby improving heating release efficiency of adsorbed materials. The taken thermally conductive material may be subjected to high-temperature purification and puffing treatment, and a heating temperature of the high-temperature purification and puffing treatment is 800°C-1500°C. For example, a temperature of high-temperature purification and puffing may be controlled at 800°C, 850°C, 900°C, 950°C, 1000°C, 1050°C, 1100°C, 1150°C, 1200°C, 1300°C, 1400°C, 1450°C, and 1500°C. This is not specifically limited. This treatment removes impurities in the thermally conductive material, increases the porosity of the thermally conductive material, is conducive to improving thermal conduction efficiency of the thermally conductive material, and facilitates subsequent filling and mixing with various components.

In a specific embodiment, in step S1, 0-8 parts by mass of an electromagnetic induction material are added, and the parts by mass of the electromagnetic induction material are controlled to be 0 parts, 0.1 parts, 0.5 parts, 1 part, 2 parts, 3 parts, 4 parts, 5 parts, 6 parts, 7 parts, 8 parts, and the like. This is not specifically limited. An aerosol generation apparatus has a magnetic field generation unit, and the electromagnetic induction material is one or a combination of a plurality of iron, nickel, copper, and germanium. A particle size of the electromagnetic induction material is 50 nm, 80 nm, 90 nm, 100 nm, 200 nm, 300 nm, 400 nm, 500 nm, 600 nm, 700 nm, 900 nm, 1 µm, or the like. This is not specifically limited. The particle size of the electromagnetic induction material is controlled to be within the foregoing disclosed range, thereby facilitating heating by the magnetic field generation unit, and heating the aerosol-generating material to generate aerosol. Step S1 further includes performing crushing treatment on the electromagnetic induction material. The crushing treatment enables the electromagnetic induction material to form a filamentous fiber with a length of 10 µm-50 µm, for example, to form a filamentous fiber with a length of 10 µm, 15 µm, 20 µm, 25 µm, 30 µm, 35 µm, 40 µm, 45 µm, or 50 µm. A length and a form of a treated material are controlled to be within the foregoing ranges, so that fibers of the electromagnetic induction material interconnect with each other to form a mesh-shaped induction heating structure, thereby increasing an induction heating area and improving uniformity of heat distribution.

In a specific embodiment, in step S1, 0-8 parts by mass of a resistance heating material are further added, and the parts by mass of the resistance heating material are controlled to be 0 parts, 0.1 parts, 0.5 parts, 1 part, 2 parts, 3 parts, 4 parts, 5 parts, 6 parts, 7 parts, 8 parts, and the like. This is not specifically limited. The resistance heating material includes at least one of zirconia, a carbon nanotube, nickel, chromium, and iron. The resistance heating material is used in a resistance-heated substrate precursor. The foregoing resistance heating materials have relatively good resistive heating efficiency, which enables rapid heating, so that heat is conducted rapidly to the tobacco, the aromatic plant, or the mixture of the two, and the tobacco, the aromatic plant, or the mixture of the two is enabled to produce aerosol, thereby rapidly generating aerosol.

S2. Perform pressing and forming: adding the substrate precursor to a mold, where there is a vertical rod in lower punch space of the mold; and pressing by an upper punch and demolding. Under an action of a pressure, a compression volume ratio is 6:1-10:3, for example, the compression volume ratio is 6:1, 4:1, 10:3, or the like. This is not specifically limited. A substrate intermediate with at least one axial air channel hole is formed. In the lower punch space of the mold, there is at least one vertical rod. An axial air channel hole adapted to a shape of the rod is pressed out after pressing of the upper punch. In other words, the substrate intermediate may have a single air channel hole or a plurality of air channel holes. This is not specifically limited herein. An outer surface of the aerosol generation substrate is cylindrical or flat-mouth-shaped (ellipsoidal), and a structure of the air channel hole may be a columnar structure, a trumpet-shaped structure with an upward opening, or another structure. This is not limited herein. The aerosol generation substrate in a hollow form has a low retention rate for aerosol. This facilitates releasing of aerosol. Therefore, compared to a granular aerosol generation substrate, the aerosol generation substrate of this application has a better aerosol release effect.

In step S2, a shape of the air channel hole may be a circular hole with equal perimeters at two ends or a square. Alternatively, an end face may be uniformly divided into a plurality of equal square bodies, or a trumpet-shaped structure with proportionally reduced or enlarged perimeters, or a stepped reduced structure.

S3. Perform drying and puffing treatment: performing secondary drying and puffing treatment on the substrate intermediate formed in step S2 to form the aerosol generation substrate, where a wall material of the aerosol generation substrate is of a porous skeleton structure including continuous micropores, where an aperture of the micropores is 10 nm-20 µm, and a porosity is 20%-80%. In an embodiment, the aperture of the micropores is 10 nm-50 nm. In this application, the aperture of the micropore is controlled to be 10 nm, 15 nm, 20 nm, 25 nm, 30 nm, 35 nm, 40 nm, 45 nm, 50 nm, 100 nm, 200 nm, 300 nm, 400 nm, 500 nm, 600 nm, 700 nm, 800 nm, 900 nm, 1 µm, 2 µm, 3 µm, 4 µm, 5 µm, 6 µm, 7 µm, 8 µm, 9 µm, 10 µm, 11 µm, 12 µm, 13 µm, 14 µm, 15 µm, 16 µm, 17 µm, 18 µm, 19 µm, 20 µm, and the like. For example, the porosity may be 20%, 30%, 40%, 45%, 50%, 55%, 60%, 65%, 70%, 75%, 80%, and the like. This is not specifically limited.

The micropores are used for aerosol formation, and pore sizes of the micropores are positively correlated with particle sizes of the aerosol. The micropores are randomly arranged and interconnected, so that the wall material forms the porous skeleton structure including the continuous micropores. This ensures that the wall material has structural strength and increases a contact area between external air and aerosol, thereby implementing more even mixing. In addition, these micropores are not voids stacked between particles in a conventional technology. These voids are usually relatively large, and usually reach 20 µm-1000 µm. The voids formed by stacking particles may decrease in volume as active components in aerosol-generating particles are released due to heating. Consequently, the overall volume of an aerosol-generating substrate shrinks and decreases, and a problem of uneven heat distribution accordingly occurs, thereby resulting in a problem of poor consistency in active components in the aerosol-generating substrate between an initial and later stages of releasing. In addition, an aerosol release channel is blocked in a procedure of volume changes, thereby affecting the overall aerosol formation efficiency. In contrast, the micropores in this application are microscopic pores created by artificial intervention, with relatively regular distribution, and present a regular polyhedral structure, a cellular structure, or another structure. The aperture is controllable within 10 nm-20 µm, and the micropores are integrally formed and interconnected in a microscopic state, and serve as aerosol formation channels. The aperture is positively correlated with a particle size of aerosol. In this application, when the aerosol generation substrate is placed inside the aerosol generation apparatus, in a heating procedure, aerosol is generated between the micropores and diffuses to a central air channel under an inhalation force of the user, and is then inhaled out through an inhalation end. Aerosol is rich during inhalation, and there is no significant difference between inhalations. In addition, the preparation method in this application does not require a plurality of high-temperature treatment processes, and a reaction condition is relatively mild and easy to control. This prevents high temperatures from destroying a flavor substance, a flavor additive, an aerosol-forming agent, and the like in tobacco or another aromatic plant, and taste is mellower, thereby improving taste experience of the user.

In a specific embodiment, in step S1, the solvent is water and/or ethanol. In a solvent system (including a solvent system with water as a dispersant, a solvent system with ethanol as a dispersant, and a solvent system formed by a mixture of water and ethanol), the polyol aerosol-forming agent combines with exposed hydroxyl groups of the binder through hydroxyl groups. In addition, water molecules in a dispersion system are accordingly transformed into a bound state. An overall state of a mixture changes from a liquid state to a solid state. The solid mixture is then mixed with another component to form a slurry, and is granulated. In step S2, pressing and forming is performed. In step S3, low-temperature vacuum drying and puffing is adopted, and the solvent in the system overflows in an order of boiling points under low-temperature vacuum to form pores, so that the wall material of the aerosol generation substrate forms the porous skeleton structure including the continuous micropores, to finally obtain the aerosol generation substrate.

In an embodiment, process parameters of low-temperature vacuum drying and puffing are: a pressure of 15 kPa-85 kPa, and a temperature of 30°C-80°C. A mass percentage content of a liquid phase component of the formed aerosol generation substrate is less than or equal to 5%, for example, the mass percentage content of the liquid phase component is 5%, 4.5%, 4%, 3.5%, 3%, 2.5%, 2%, 1.5%, 1%, 0.9%, and the like. A pressure parameter of low-temperature vacuum drying is controlled to be 15 kPa, 20 kPa, 25 kPa, 30 kPa, 35 kPa, 40 kPa, 50 kPa, 55 kPa, 60 kPa, 65 kPa, 70 kPa, 75 kPa, 80 kPa, 85 kPa, and the like. This is not specifically limited. A drying temperature is controlled to be 30°C, 35°C, 40°C, 45°C, 50°C, 55°C, 60°C, 65°C, 70°C, 75°C, and 80°C. This is not specifically limited. A reaction condition for low-temperature vacuum drying in this application is relatively mild, so that a pore-forming agent such as water or ethanol can be fully dried and evaporated, to form a dense interconnected pore structure. This can further avoid flavor evaporation or damage to a flavor substance due to high-temperature baking, and taste is mellower, thereby improving taste experience of the user. Herein, the "liquid phase component" includes solvents such as water and ethanol, and liquid phase components included in the aerosol-forming agent, the binder, and the like, and is not limited to only water.

In a specific embodiment, in step S1, the solvent is water and/or ethanol. In a solvent system, the polyol aerosol-forming agent combines with exposed hydroxyl groups of the binder through hydroxyl groups. In addition, water molecules in a dispersion system are accordingly transformed into a bound state. An overall state of a mixture changes from a liquid state to a solid state. The solid mixture is then mixed with another component to form a slurry, and is granulated. In step S2, pressing and forming is performed. In step S3, hot-air drying and puffing is adopted, and the solvent in the system overflows in an order of boiling points under a hot-air drying condition to form pores, so that the wall material of the aerosol generation substrate forms the porous skeleton structure including the continuous micropores, to finally obtain the aerosol generation substrate.

In an embodiment, a process parameter of hot-air drying and puffing is 50°C-120°C. For example, a temperature of hot-air drying is controlled to be 50°C, 55°C, 60°C, 65°C, 70°C, 75°C, 80°C, 90°C, 100°C, 110°C, 120°C, and the like. This is not specifically limited. A mass percentage content of a liquid phase component of the formed aerosol generation substrate is less than or equal to 5%, for example, the mass percentage content of the liquid phase component is 5%, 4.5%, 4%, 3.5%, 3%, 2.5%, 2%, 1.5%, 1%, 0.9%, and the like. A reaction condition for hot-air drying and puffing in this application is relatively mild and easy to control, so that a pore-forming agent such as water or ethanol can be fully dried and evaporated, to form a dense interconnected pore structure. This can further avoid flavor evaporation or damage to a flavor substance due to high-temperature baking, and taste is mellower, thereby improving taste experience of the user.

In a specific embodiment, when the solvent added in step S1 is water and does not include ethanol, the polyol aerosol-forming agent combines with exposed hydroxyl groups of the binder through hydroxyl groups under an aqueous condition. In addition, water molecules in a dispersion system are accordingly transformed into a bound state. An overall state of a mixture changes from a liquid state to a solid state. The solid mixture is then mixed with another component to form a slurry, and is granulated. In step 2, pressing and forming is performed. In step 3, a freeze-drying process is adopted, and an aqueous ice crystal is transformed into a free water molecule through sublimation drying to overflow to form pores, so that the wall material of the aerosol generation substrate forms the porous skeleton structure including the continuous micropores, to finally obtain the aerosol generation substrate. In this application, the freeze-drying process is adopted, ice crystals may be formed according to different freezing points of the mixture. After the water molecules in the mixture are transformed into a bound state, recrystallization of aqueous ice crystals may be inhibited, achieving an effect of uniform ice crystal distribution. In addition, according to a principle of "expansion upon freezing and contraction upon warming" of water, puffing of a formed substrate is achieved. Finally, according to a principle of sublimation drying, the aqueous ice crystals are transformed into free water molecules to overflow. By using the freeze-drying process, an effect of uniformly distributed micropores is achieved through freeze crystallization.

In an embodiment, a process parameter of the freeze-drying process is -10°C to - 87°C. For example, a process parameter of freeze-drying is controlled to be -10°C, -12°C, -15°C, -18°C, -20°C, -22°C, -25°C, -30°C, -35°C, -40°C, -45°C, -50°C, -55°C, -60°C, -65°C, -70°C, -75°C, -80°C, -85°C, -87°C, or the like. A pre-freezing temperature, a primary drying temperature, and a desorption drying temperature are controlled within this range, and an actual drying temperature may be appropriately modified as needed. This is not specifically limited. In this case, a mass percentage content of a liquid phase component of the formed aerosol generation substrate is less than or equal to 5%, for example, the mass percentage content of the liquid phase component is 5%, 4.5%, 4%, 3.5%, 3%, 2.5%, 2%, 1.5%, 1%, 0.9%, and the like. A reaction condition for hot-air drying and puffing in this application is relatively mild and easy to control, so that a pore-forming agent such as water or ethanol can be fully dried and evaporated, to form a dense interconnected pore structure. This can further avoid flavor evaporation or damage to a flavor substance due to high-temperature baking, and taste is mellower, thereby improving taste experience of the user.

This application further provides an aerosol generation substrate, where the aerosol generation substrate has at least one air channel hole running through two ends, a wall material of the aerosol generation substrate is of a porous skeleton structure including continuous micropores, and an aperture of the micropore is 10 nm-20 µm, and a porosity is 20%-80%. In this application, the aperture of the micropore is controlled to be 10 nm, 15 nm, 20 nm, 25 nm, 30 nm, 35 nm, 40 nm, 45 nm, 50 nm, 100 nm, 200 nm, 300 nm, 400 nm, 500 nm, 600 nm, 700 nm, 800 nm, 900 nm, 1 µm, 2 µm, 3 µm, 4 µm, 5 µm, 6 µm, 7 µm, 8 µm, 9 µm, 10 µm, 11 µm, 12 µm, 13 µm, 14 µm, 15 µm, 16 µm, 17 µm, 18 µm, 19 µm, 20 µm, and the like. For example, the porosity is 20%, 30%, 40%, 45%, 50%, 55%, 60%, 65%, 70%, 75%, 80%, and the like. This is not specifically limited. The micropores are randomly arranged and interconnected, so that the wall material forms the porous skeleton structure including the continuous micropores. This ensures that the wall material has structural strength and increases a contact area between external air and aerosol, thereby implementing more even mixing. In a heating procedure, aerosol is generated between the micropores and diffuses to a central air channel under an inhalation force of a user, and is then inhaled out through an inhalation end. Aerosol is rich during inhalation, and there is no significant difference between inhalations.

The following describes this application by using specific embodiments.

### Embodiment 1

A method for preparing an aerosol generation substrate includes the following steps:
S1. Prepare a substrate precursor: taking 55 parts of tobacco and 10 parts of aromatic plant (mint) to form a mixture, and performing impact crushing treatment on the mixture until a material obtained through crushing treatment becomes a particle in a shape of a spindle and/or a polyhedron, where an aspect ratio of the spindle or the polyhedron is approximately 3:1, and a particle size of the spindle or the polyhedron is approximately 18 µm; placing a treated mixture in a vacuum-sealed environment, and adding an acidic treatment solution (a benzoic acid solution) to achieve a final pH of 6.8 of a treatment system; and performing heating and aroma-producing treatment at a heating temperature of 60°C for a heating time of 20 minutes; and
   taking the foregoing mixture of the tobacco and the aromatic plant, 10 parts of an inorganic porous material (zeolite), 5 parts of a flavor additive (rose essence), 2 parts of a binder (pullulan), and 15 parts of a polyol aerosol-forming agent (glycerol), adding water as a solvent, and performing slurry preparation, granulation, and preliminary drying to form a basic particle, where a viscosity of the basic particle is 500 Pa·s, and a mass percentage content of a liquid phase component is 10%, thereby obtaining the substrate precursor.
S2. Perform pressing and forming: adding the substrate precursor to a mold, where there is a vertical rod in lower punch space of the mold; and pressing by an upper punch and demolding, where under an action of a pressure, a compression volume ratio is 6:1, to form a substrate intermediate with one air channel hole.
S3. Perform drying and puffing treatment: performing secondary drying and puffing treatment on an aerosol generation substrate formed in step S2, for example, low-temperature vacuum drying and puffing. Process parameters of low-temperature vacuum drying and puffing are: a pressure of 15 kPa and a temperature of 80°C. An aerosol generation substrate with a porous skeleton structure as a wall material is formed. A mass percentage content of a liquid phase component of the aerosol generation substrate is approximately 4.9%, as shown in FIG. 2.

The aromatic plant may be replaced with at least one of the aromatic plants disclosed above. The acidic treatment solution may be replaced with at least one of citric acid, lactic acid, levulinic acid, salicylic acid, and tartaric acid, or a mixture thereof with benzoic acid. The foregoing zeolite may be replaced with at least one of molecular sieve, diatomaceous earth, montmorillonite, alumina, silica gel, activated carbon, calcium silicate, a chitosan porous material, cellulose fiber, a lignin particle, clay, sepiolite, and palygorskite, or a mixture thereof with zeolite. The rose essence may be replaced with another essence. The foregoing pullulan may be replaced with at least one of tamarind polysaccharide and hydroxypropyl methylcellulose, or a mixture thereof with pullulan. The foregoing glycerol may be replaced with at least one of propylene glycol, butylene glycol, and butanetriol, or a mixture thereof with glycerol.

### Embodiment 2

A method for preparing an aerosol generation substrate includes the following steps:
S1. Prepare a substrate precursor: taking 50 parts of tobacco and 30 parts of aromatic plant (mint), 20 parts of an inorganic porous material (10 parts of zeolite and 10 parts of montmorillonite), 10 parts of a flavor additive (lily essence), 1 part of a binder (pullulan), and 30 parts of a polyol aerosol-forming agent (glycerol), adding ethanol, and performing slurry preparation, granulation, and preliminary drying to form a basic particle, where a viscosity of the basic particle is 1000 Pa·s, and a mass percentage content of a liquid phase component is 25%, thereby obtaining the substrate precursor.
S2. Perform pressing and forming: adding the substrate precursor to a mold, where there are three vertical rods in lower punch space of the mold; and pressing by an upper punch and demolding, where under an action of a pressure, a compression volume ratio is 4:1, to form a substrate intermediate with three air channel holes.
S3. Perform drying and puffing treatment: performing secondary drying and puffing treatment on an aerosol generation substrate formed in step S2, for example, low-temperature hot-air drying and puffing. A process parameter of hot-air drying and puffing is 50°C, an aerosol generation substrate with a mass percentage content of a liquid phase component of approximately 4.5% is formed, and a wall material of the aerosol generation substrate is of a porous skeleton structure including continuous micropores.

### Embodiment 3

A method for preparing an aerosol generation substrate includes the following steps:
S1. Prepare a substrate precursor: taking 25 parts of tobacco and 5 parts of aromatic plant (mint), 15 parts of an inorganic porous material (10 parts of zeolite and 5 parts of montmorillonite), 7 parts of a flavor additive (lily essence), 5 parts of a binder (pullulan), and 10 parts of a polyol aerosol-forming agent (glycerol), adding 3 parts of an electromagnetic induction material (iron powder), adding water as a solvent, and performing slurry preparation, granulation, and preliminary drying to form a basic particle, where a viscosity of the basic particle is 1500 Pa·s, and a mass percentage content of a liquid phase component is 50%, thereby obtaining the substrate precursor.
S2. Perform pressing and forming: adding the substrate precursor to a mold, where there is one vertical rod in lower punch space of the mold; and performing pressing by an upper punch and demolding, where under an action of a pressure, a compression volume ratio is 10:3, to form a substrate intermediate with one air channel hole.
S3. Perform drying and puffing treatment: performing secondary drying and puffing treatment on an aerosol generation substrate formed in step S2, for example, a freeze-drying process. A process parameter of the freeze-drying process is -10°C to -87°C, an aerosol generation substrate with a mass percentage content of a liquid phase component of approximately 1.2% is formed, and a wall material of the aerosol generation substrate is of a porous skeleton structure including continuous micropores, thereby obtaining the aerosol generation substrate.

### Comparative Example 1

In Comparative Example 1, all steps, process parameters, formulation ratios, and the like are the same as those in Embodiment 1, except that impact crushing treatment, heating treatment, and treatment with an acid treatment solution are not performed on tobacco and an aromatic plant in step S1.

### Comparative Example 2

In Comparative Example 2, all steps, process parameters, formulation ratios, and the like are the same as those in Embodiment 1, except that process parameters of vacuum drying adopted in step S3 are different from those in Embodiment 1. The process parameters of vacuum drying adopted in Comparative Example 2 are 100°C and 90 kPa.

### Comparative Example 3

In Comparative Example 3, all steps, process parameters, formulation ratios, and the like are the same as those in Embodiment 2, except that a process parameter of hot-air drying adopted in step S3 is different from that in Embodiment 2. The process parameter of hot-air drying adopted in Comparative Example 3 is 150°C.

### Comparative Example 4

In Comparative Example 4, all steps, process parameters, formulation ratios, and the like are the same as those in Embodiment 3, except that a process parameter of freeze-drying adopted in step S3 is different from that in Embodiment 3. The process parameter of freeze-drying adopted in Comparative Example 4 is -20 to 20°C.

### Comparative Example 5

A method for preparing an aerosol generation substrate includes the following steps:
taking 55 parts of tobacco and 10 parts of aromatic plant (mint) to crush into powder; then mixing with 10 parts of an inorganic porous material (zeolite), 5 parts of a flavor additive (rose essence), 2 parts of a binder (pullulan), and 15 parts of a polyol aerosol-forming agent (glycerol); performing molding by injection molding or compression molding; and cutting into sections, and performing drying to obtain an aerosol generation substrate. The aerosol generation substrate is scanned by using a scanning electron microscope, and it is found that a porous skeleton structure including continuous micropores is not formed on a wall material of the aerosol generation substrate.

The aerosol generation substrates from Embodiments 1-3 and Comparative Examples 1-5 are subjected to performance tests. Test standards are in accordance with ISO 20778:2018 Cigarettes - Routine analytical cigarette smoking machine - Definitions and standard conditions with an intense smoking regime; YC/T 138 Tobacco and tobacco products - The sensory evaluation methods; and YC/T 156 Cigarettes - Determination of nicotine in smoke condensates - Gas-chromatographic method. Test results are shown in Table 1.

**Table 1. Performance test results of aerosol generation substrates from Embodiments 1-3 and Comparative Examples 1-5**

| Embodiment/ Comparative Example | Aerosol amount (mg) | Nicotine in aerosol (mg) | Aroma feature (30 points) | Aerosol feature (25 points) | Taste feature (30 points) | Consistency feature (15 points) | Overall sensory score (100 points) |
|---|---|---|---|---|---|---|---|
| Embodiment 1 | 32 | 1.2 | 25 | 20 | 26 | 13 | 84 |
| Embodiment 2 | 31 | 1.1 | 24 | 21 | 24 | 14 | 83 |
| Embodiment 3 | 31.6 | 1.3 | 26 | 21 | 25 | 13 | 85 |
| Comparative Example 1 | 30 | 1.5 | 22 | 20 | 23 | 12 | 77 |
| Comparative Example 2 | 30.2 | 1.4 | 22 | 20.5 | 23 | 11 | 76.5 |
| Comparative Example 3 | 31 | 1.3 | 21 | 20.5 | 22.5 | 12 | 76 |
| Comparative Example 4 | 30 | 1.3 | 21.5 | 20 | 22 | 12 | 75.5 |
| Comparative Example 5 | 25 | 0.7 | 15 | 16 | 20 | 7 | 58 |

It may be learned from the test results of the aerosol generation substrates of Embodiment 1 to Embodiment 3 and Comparative Example 1 to Comparative Example 5 that in this application, the tobacco and/or the aromatic plant are crushed, acid is added, and vacuum heating treatment is performed. This is conducive to reducing irritation, thereby achieving a purpose of disrupting cell walls and transferring flavor substances inside the cells to surfaces. In this way, during heat-not-burn, aroma is more easily released, and flavor is richer and mellower, thereby improving taste experience of the user. In this application, the pore-forming agent such as water or ethanol is added in a preparation procedure, and secondary drying is performed on the substrate intermediate, so that the wall material forms the porous skeleton structure including the continuous micropores. This ensures structural strength and increases a contact area between external air and aerosol, so that the aerosol is more evenly mixed and the aerosol is abundant during inhalation.

It may be learned from Comparative Example 1 that not performing the aroma-producing pretreatment on the tobacco and the aromatic plant is inconducive to releasing aroma, affecting taste experience. It may be learned from Comparative Example 2 that using an inappropriate parameter of vacuum drying may lead to volatilization of an aroma-producing substance, and destroy a structure of the aroma-producing substance, which is not conducive to forming the porous skeleton structure including the continuous micropores on the wall material of the aerosol generation substrate, affecting taste experience. It may be learned from Comparative Example 3 that using an inappropriate parameter of hot-air drying may also lead to volatilization of an aroma-producing substance, and destroy a structure of the aroma-producing substance, which is not conducive to forming the porous skeleton structure including the continuous micropores on the wall material of the aerosol generation substrate, affecting taste experience. It may be learned from Comparative Example 4 that using an inappropriate parameter of freeze-drying may also lead to volatilization of an aroma-producing substance, and destroy a structure of the aroma-producing substance, which is not conducive to forming the porous skeleton structure including the continuous micropores on the wall material of the aerosol generation substrate, affecting taste experience. It may be learned from Comparative Example 5 that not adding a pore-forming agent and not performing secondary drying on the substrate intermediate leads to the wall material of the aerosol generation substrate being unable to form the porous skeleton structure including the continuous micropores, or the porous skeleton structure cracking, which severely affects aerosol release and an aroma feature, thereby affecting taste experience.

## Claims

1. A method for preparing an aerosol generation substrate, comprising the following steps:
preparing a substrate precursor:
taking pretreated tobacco and/or an aromatic plant, an inorganic porous material, a polyol aerosol-forming agent, a flavor additive, and a binder, adding a solvent, wherein the solvent is water and/or ethanol, and performing slurry preparation, granulation, and preliminary drying to form a basic particle, thereby obtaining the substrate precursor;
performing pressing and forming: adding the substrate precursor to a mold, and performing pressing and demolding, to form a substrate intermediate with at least one axial air channel hole; and
performing drying and puffing treatment: performing secondary drying and puffing treatment on the substrate intermediate formed in the step of performing pressing and forming to form an aerosol generation substrate, wherein a wall material of the aerosol generation substrate is of a porous skeleton structure comprising continuous micropores.

2. The method for preparing an aerosol generation substrate according to claim 1, wherein in the step of preparing a substrate precursor, a viscosity of the formed basic particle is 500 Pa·s-1500 Pa·s, and a mass percentage content of a liquid phase component in the substrate precursor is 10%-50%.

3. The method for preparing an aerosol generation substrate according to claim 1, wherein in the step of preparing a substrate precursor, pretreatment of the tobacco and/or the aromatic plant comprises taking the tobacco and/or the aromatic plant for impact crushing treatment; and then placing the foregoing materials in a vacuum-sealed environment, adding an acidic treatment solution, and performing heating treatment at a heating temperature of 60°C-120°C, so that a volume of the tobacco and/or the aromatic plant expands by 1.1-1.5 times, and an amount of released free nicotine increases by at least 50%.

4. The method for preparing an aerosol generation substrate according to claim 1, wherein in the step of preparing a substrate precursor, the inorganic porous material comprises at least one of zeolite, molecular sieve, diatomaceous earth, montmorillonite, alumina, silica gel, activated carbon, calcium silicate, a chitosan porous material, a cellulose fiber, a lignin particle, clay, sepiolite, or palygorskite;
and/or, the polyol aerosol-forming agent comprises at least one of glycerol, propylene glycol, butylene glycol, and butanetriol;
and/or, the flavor additive is an extract of tobacco and/or an extract of an aromatic plant;
and/or the binder comprises one or a combination of a plurality of pullulan, tamarind polysaccharide, and hydroxypropyl methylcellulose.

5. The method for preparing an aerosol generation substrate according to claim 1, wherein in the step of preparing a substrate precursor, the preparation of the substrate precursor comprises the following raw materials in parts by mass: 30-80 parts of the tobacco and/or the aromatic plant, 10-30 parts of the polyol aerosol-forming agent, 0-5 parts of the binder, 5-20 parts of the inorganic porous material, and 5-10 parts of the flavor additive.

6. The method for preparing an aerosol generation substrate according to claim 1, wherein in the step of preparing a substrate precursor, 0-8 parts by mass of an electromagnetic induction material are further added, wherein the electromagnetic induction material is at least one of iron, nickel, copper, germanium, carbon, chromium, tin, manganese, and aluminum;
or in the step of preparing a substrate precursor, 0-8 parts by mass of a resistance heating material are further added, wherein the resistance heating material comprises at least one of zirconia, a carbon nanotube, nickel, chromium, and iron;
and/or in the step of preparing a substrate precursor, 0-5 parts by mass of a thermally conductive material subjected to high-temperature purification treatment are added, wherein the thermally conductive material is at least one of iron powder, copper powder, graphite powder, graphene, boron nitride, alumina, and carbon powder.

7. The method for preparing an aerosol generation substrate according to claim 1, wherein in the step of performing drying and puffing treatment, low-temperature vacuum drying and puffing is adopted, and the solvent in a system overflows in an order of boiling points under low-temperature vacuum to form pores, so that the wall material of the aerosol generation substrate forms the porous skeleton structure comprising the continuous micropores.

8. The method for preparing an aerosol generation substrate according to claim 7, wherein process parameters of low-temperature vacuum drying and puffing are: a temperature of 30°C-80°C, and a pressure of 15 kPa-85 kPa.

9. The method for preparing an aerosol generation substrate according to claim 1, wherein in the step of performing drying and puffing treatment, hot-air drying and puffing is adopted, and the solvent in a system overflows in an order of boiling points under a hot-air drying condition to form pores, so that the wall material of the aerosol generation substrate forms the porous skeleton structure comprising the continuous micropores.

10. The method for preparing an aerosol generation substrate according to claim 1, wherein the solvent added in the step of preparing a substrate precursor is water, in the step of performing drying and puffing treatment, a freeze-drying process is adopted, and an aqueous ice crystal is transformed into a free water molecule through sublimation drying to overflow to form pores, so that the wall material of the aerosol generation substrate forms the porous skeleton structure comprising the continuous micropores.

11. The method for preparing an aerosol generation substrate according to claim 1, wherein in the step of performing pressing and forming, by feeding the substrate precursor into the mold, under an action of a pressure, a compression polymer volume ratio is 6:1-10:3, an integrally formed substrate intermediate is demolded, there is at least one vertical rod in lower punch space of the mold, and an axial air channel hole adapted to a shape of the rod is pressed out after pressing of the upper punch.

12. The method for preparing an aerosol generation substrate according to claim 3, wherein in the step of preparing a substrate precursor, a viscosity of the formed basic particle is 500 Pa·s-1500 Pa·s, and a mass percentage content of a liquid phase component in the substrate precursor is 10%-50%.

13. The method for preparing an aerosol generation substrate according to claim 12, wherein in the step of preparing a substrate precursor, the preparation of the substrate precursor comprises the following raw materials in parts by mass: 30-80 parts of the tobacco and/or the aromatic plant, 10-30 parts of the polyol aerosol-forming agent, 0-5 parts of the binder, 5-20 parts of the inorganic porous material, and 5-10 parts of the flavor additive.

14. The method for preparing an aerosol generation substrate according to any one of claims 1 to 13, wherein in the step of performing drying and puffing treatment, the formed micropore of the aerosol generation substrate is of 10 nm-20 µm, and a porosity is 20%-80%.

15. An aerosol generation substrate, wherein the aerosol generation substrate has at least one axial air channel hole, a wall material of the aerosol generation substrate is of a porous skeleton structure comprising continuous micropores, and an aperture of the micropore is 10 nm-20 µm, and a porosity is 20%-80%.

16. The aerosol generation substrate according to claim 15, comprising the following raw materials in parts by mass: 30-80 parts of tobacco and/or an aromatic plant, 10-30 parts of a polyol aerosol-forming agent, 0-5 parts of a binder, 5-20 parts of an inorganic porous material, and 5-10 parts of a flavor additive.
